

1

3,634,239

## LUBRICANT COMPOSITIONS

Alexander C. B. MacPhail, Cheshire, England, and John E. Lauck, Godfrey, and Kenneth T. Wendler, Alton, Ill., assignors to Shell Oil Company, New York, N.Y.  
No Drawing. Filed Sept. 8, 1969, Ser. No. 856,159  
Int. Cl. C10m 1/46

U.S. Cl. 252—32.5

9 Claims

## ABSTRACT OF THE DISCLOSURE

Synthetic ester lubricating oil compositions containing minor amounts of (1) a trihydrocarbyl phosphate, (2) an alkyl amine salt of a monohaloalkylphosphonic acid and (3) a dicarboxylic acid have improved anticorrosion, anti-oxidation and load-carrying properties.

This invention relates to synthetic ester lubricating oils having excellent corrosion resistance, oxidation stability and load-carrying properties. More particularly it relates to synthetic ester oils containing a combination of (1) a trihydrocarbyl phosphate, (2) an alkyl amine salt of a monohaloalkylphosphonic acid and (3) a dicarboxylic acid.

Synthetic ester base oils are particularly suitable for use in high temperature-high speed lubricating applications such as in the lubrication of gas turbine engines because of their inherently good thermal stability and desirable viscosity properties. Although ester base lubricants are superior to mineral lubricating oils in many respects, they have a tendency to be slightly more corrosive and will undergo oxidation and decompose at elevated temperatures. It is known that the thermal decomposition of synthetic ester oils is significantly accelerated by the presence of minute quantities of dissolved metals such as iron which can result from the dissolution of steel components by the ester base stocks or additives incorporated into these oils.

Concern over the problem of corrosion and catalytic degeneration is reflected in the recently proposed military specification for aircraft gas turbine lubricants, MIL-L-23699B. This specification contains a number of tests directed to evaluating the corrosivity and oxidation-resistance of lubricating fluids, including a newly developed Naval Thermal Stability-Corrosivity test. The demands placed on lubricating oils by this specification are extremely stringent, and only compositions possessing exceptional properties can qualify. Such lubricant compositions are the subject of the present invention.

It has now been found that lubricant compositions comprising a major amount of a synthetic ester lubricating oil and minor amounts each of (1) a trihydrocarbyl phosphate, (2) an alkyl amine salt of a monohaloalkylphosphonic acid and (3) a dicarboxylic acid have excellent anticorrosion, antoxidation and load-carrying properties. The aforementioned compositions have been found to be remarkably effective in passivating steel surfaces, thus substantially preventing dissolution of the metal, which correspondingly also increases the oxidation stability of the oil. In addition, the present compositions have been found to possess excellent load-carrying properties and are eminently suited for use in high temperature-high speed lubricating applications.

The hydrocarbyl groups can be alkyl, aryl, alkaryl and aralkyl and templated for use in the present compositions include those represented by the formula:



2

wherein  $R_1$ ,  $R_2$  and  $R_3$  are the same or different hydrocarbyl groups having from 1 to about 15 carbon atoms. The hydrocarbyl groups can be alkyl, aryl, alkaryl and aralkyl radicals. Aryl or alkaryl groups having from 1 to 10 carbon atoms are especially preferred.

Examples of suitable trihydrocarbyl phosphate compounds include tricresyl phosphate, tri(2,4-dimethylphenyl) phosphate, tri(p-ethylphenyl) phosphate, tri-(2-methyl-4-isopropylphenyl) phosphate, tri(p-tert butylphenyl) phosphate, tri-(2,6 - dimethyl - 4-tert-butylphenyl) phosphate, tri - (4 - methyl-1-naphthyl)phosphate, ethyl di(p-cresyl) phosphate, 2,6-xylenyl di-(n-butyl) phosphate, triphenyl phosphate, cresyl diphenyl phosphate, dicresyl phenyl phosphate, xylyl dicresyl phosphate, trixylyl phosphate, dimethyl xylyl phosphate, dimethyl tolyl phosphate, dimethyl phenyl phosphate, methyl diphenyl phosphate, octyl diphenyl phosphate, trimethyl phosphate, triethyl phosphate, tri-n-butyl phosphate, tris(2-ethyl hexyl) phosphate, and mixtures thereof. Of the foregoing, tricresyl phosphate has been found to be particularly advantageous for use in the compositions of the invention.

Amine salts which are suitable for use in the present compositions are the salts of  $C_{8-30}$  alkyamines and monohaloalkylphosphonic acids. Haloalkylphosphonic acid which can be used in forming these salts have the general formula



wherein R is a monohaloalkyl group containing 1 to 4, preferably 1 to 2 carbon atoms. Preferred halogens are fluorine, chlorine and bromine. Acids wherein the R group contains a chlorine atom substituted on the alpha carbon atom are especially advantageous for the purposes of the invention. Examples of such acids, include monochloromethylphosphonic acid,  $\alpha$ -monochloroethylphosphonic acid,  $\alpha$ -monochloropropylphosphonic acid,  $\alpha$ -chloro- $\alpha$ -methyl-ethylphosphonic acid,  $\alpha$ -chloro-butylphosphonic acid and  $\alpha$ -chloro- $\alpha$ -methyl-propylphosphonic acid. The anhydrides of the aforementioned acids can also be used to prepare suitable amine salts.

Amines which form effective salts with the above-described acids are primary or secondary alkyl amines having at least 8, preferably 8 to 30, and more preferably 12 to 24 carbon atoms per molecule. Branched tertiary-alkyl primary amines are preferred; "branched" in this context means having at least 2 hydrocarbon substituents attached to the main carbon chain. As the tertiary-alkyl radical, the radical of polyisobutylene and polypropylene, and mixtures of these are particularly preferred. Examples of these amines are 1,1,3,3-tetramethylbutylamine, 1,1,3,3,5,5-hexamethylhexylamine, 1,1,3,3,5,5,7,7-octamethyl-octylamine and 1,1,3,3,5,5,7,7,9,9-decamethyldecylamine. Tertiary alkyl methyl primary amines, such as 2,2,4,4-tetramethylpentylamine and 2,2,4,4,6,6-hexamethyl hexylamine are also suitable.

Other primary amines having 8 to 30 carbons which are appropriate for forming the salts of the invention are described in Bortnick, U.S. 2,606,923, issued Aug. 12, 1952, and Bortnick, U.S. 2,611,782, issued Sept. 23, 1952. These include tert-tridecylamine,



as well as isoheptyl diethyl carbonylamine, isoocetyl ethyl propylcarbonylamine, etc. Primary amines of this type are commercially available from Rohm and Haas Company under the trade name of "Primenes." The amine may also be a polyamine, such as a diamine or triamine, and

may contain other non-reactive groups, such as amide or ether groups in the carbon chain.

Some specific examples of secondary amines for making the phosphonic acid salts are diethylamine, dihexylamine, di(2-ethylhexyl)amine, dioctylamine, didecylamine, di-dodecylamine, ditetradecylamine, dihexadecylamine, di-octadecylamine, dibromooctadecylamine, isopropylol-ylamine, diricinoleylamine, butyricinoleylamine, butyl-2-ethylhexylamine, dilaurylamine, methyloleylamine, ethyl-octylamine, isoamylhexylamine, dicyclohexylamine, dicyclopentylamine, cyclohexyloctylamine, cyclohexylbenzyl-amine, benzylcetylamine, benzyl-2-ethylhexylamine, allyl-octylamine, dodecyl-2-ethylhexylamine, N,N-diallyl trimethylene diamine, 3-hexyl-morpholine, and the like.

The phosphonic acid-amine salts for use in the invention can be prepared by direct neutralization of haloalkyl-phosphonic acid with a substantially stoichiometric amount of amine. The reaction occurs at normal or moderately elevated temperatures and may be carried out in the presence of an inert diluent or solvent, such as a hydrocarbon, alcohol, ether, ketone, etc. Preparation of these salts is described in Watson et al., U.S. 2,858,332, issued Oct. 28, 1958.

The phosphonic acid-amine salts useful in the invention may also be modified with an alkali metal as described in Price et al., U.S. 3,112,267, issued Nov. 26, 1963. The full amine salt of the phosphonic acid is prepared and is then treated in a low-boiling solvent with an alkali metal hydroxide, carbonate, or alcoholate such that one of the amine groups is replaced with an alkali metal. Preferred alkali metals are sodium, potassium, and lithium.

Dicarboxylic acids which can be effectively used in combination with the previously described trihydrocarbyl phosphates and amine salts are those dicarboxylic acids having from 4 to 14 carbon atoms. While it is contemplated that other dicarboxylic acids can be used, aliphatic dicarboxylic acids are preferred. Examples of these include adipic, pimelic, suberic, azelaic, sebacic, brassylic, and the like. Azelaic acid has been found to be particularly effective in the compositions of the invention.

Suitable synthetic lubricant base stocks for the practice of the invention are esters of alcohols having 1 to 20, especially 4 to 12 carbon atoms and aliphatic carboxylic acids having from 3 to 20, especially 4 to 14 carbon atoms. The ester base may comprise a simple ester (reaction product of a monohydroxyalcohol and a monocarboxylic acid) a polyester (reaction product of an alcohol and an acid, one of which has more than one functional group), or a complex ester (reaction product of a poly-functional acid with more than one alcohol, or of a poly-functional alcohol with more than one acid). Also, excellent synthetic lubricants may be formulated with mixtures of esters, such as major proportions of complex esters and minor amounts of diesters.

Examples of suitable ester base oils are ethyl palmitate, 55 ethyl laurate, butyl stearate, di-(2-ethylhexyl)sebacate, di-(2-ethylhexyl) azelate, ethyl glycol dilaurate, di-(2-ethylhexyl)phthalate, di-(1,3-methylbutyl) adipate, di(1-ethylpropyl) azelate, diisopropoxylate, dicyclohexyl sebacate, glycerol tri-n-heptoate, di(undecyl) azelate, and tetraethylene glycol di-(2-ethylene caproate), and mixtures thereof. A preferred mixture of such esters consists of about 50-80% bis (2,2,4-trimethylpentyl) azelate and 20 to 50% 1,1,1-trimethyl propane triheptanoate.

Especially preferred esters for use as base stocks in the present invention are esters of monocarboxylic acids having 4 to 14 carbons and polyalcohols such as pentaerythritol, dipentaerythritol, and trimethylolpropane. Examples of these esters are pentaerythritol tetrabutyrate, pentaerythritol tetravalerate, pentaerythritol tetracaproate, pentaerythritol dibutyratedicaproate, pentaerythritol butyratecaproate divalerate, pentaerythritol butyrate trivalerate, pentaerythritol butyrate tricaproate, pentaerythritol tributyratcaproate, mixed C<sub>4-10</sub> saturated fatty acid esters of pentaerythritol, dipentaerythritol hexavalerate,

dipentaerythritol hexacaproate, dipentaerythritol hexaheptoate, dipentaerythritol hexacaprylate, dipentaerythritol tributyratetraproate, dipentaerythritol trivalerate tri-pelargonate dipentaerythritol mixed hexaesters of C<sub>4-10</sub> fatty acids and trimethylolpropane heptoate. Mixtures of C<sub>4-10</sub> monocarboxylic acid esters of pentaerythritol and dipentaerythritol are particularly advantageous base oils and are commercially available from Hercules, Inc.

The trihydrocarbyl phosphate is employed in the present 10 compositions in amounts of from 0.005 to 10% by weight, preferably from 0.01 to 3% based on the total composition weight. The amine salt of the monohaloalkylphosphonic acid can be used in amounts of from 0.005% to 10% by weight, but preferably is employed in the 15 amounts of from 0.01 to 2% by composition weight. The dicarboxylic acid constituent is generally present in quantities of from 0.001 to 2% by weight, preferably from 0.005 to 0.1% by composition weight.

Other additives can also be incorporated into the 20 compositions according to the invention. Examples of such additives are viscosity index improvers, e.g. methacrylate polymers and copolymers; antioxidants, e.g. aryl amines, phosphorous compounds or phenolic compounds; and corrosion inhibitors, antifoam agents, detergents or any other additive recognized in the art to perform a particular function or functions.

The invention will be further described by means of the 25 following examples. It should be understood, however, that these examples are given for illustrative purposes only and the invention in its broader aspects is not limited thereto.

#### EXAMPLE I

To illustrate the ester base compositions of the present 30 invention, compositions II, VI, IX, and X were formulated as shown in Table I and thereafter compared with compositions I, III, IV, V, VII, and VIII (not in accordance with the invention) by means of one or more of the test procedures hereinafter described.

TABLE I

|              | Base oil | Additive |       |       |
|--------------|----------|----------|-------|-------|
|              |          | A        | B     | C     |
| Composition: |          |          |       |       |
| I            | R        | 0.20     | ----- | ----- |
| II           | Q        | 0.17     | 1.0   | 0.02  |
| III          | P        | -----    | 1.22  | ----- |
| IV           | P        | 1.22     | ----- | ----- |
| V            | P        | -----    | ----- | 1.22  |
| VI           | P        | 0.20     | 1.0   | 0.02  |
| VII          | V        | 0.20     | ----- | ----- |
| VIII         | S        | 0.20     | 1.0   | ----- |
| IX           | T        | 0.17     | 1.0   | 0.02  |
| X            | U        | 0.17     | 1.0   | 0.02  |

NOTES—

Additives:

Additive A=C<sub>18-22</sub> tertiary alkyl primary amine salt of monochloromethylphosphonic acid.

Additive B=Tricresyl phosphate.

Additive C=Azoleaic acid.

Base Oils:

Base Oil P=Mixed C<sub>4-10</sub> acid esters of pentaerythritol and dipentaerythritol containing 2.5% w. of amine antioxidants, 0.1% w. of triazole corrosion inhibitors, 0.25% w. of a copolymeric dispersant and 10 p.p.m. silicone fluid antifoamant.

Base Oil Q=Base oil P minus 0.025% w. triazole corrosion inhibitor.

Base Oil R=Base oil P plus 0.5% w. amine antioxidant.

Base Oil S=Mixed C<sub>4-10</sub> acid esters of pentaerythritol and dipentaerythritol containing 2.5% w. of amine antioxidants, 1% w. of a phenothiazine antioxidant, 1.0% w. of a phosphorothionate compound, 0.1% w. of triazole corrosion inhibitors and 10 p.p.m. silicone fluid antifoamant.

Base Oil T=Base Oil S minus 0.05% w. triazole corrosion inhibitor.

Base Oil U=Base Oil T minus 0.5% w. amine antioxidant.

Base Oil V=Base Oil S plus 1% w. of the amine antioxidants, minus the phosphorothionate compound.

#### EXAMPLE II

To demonstrate the effectiveness of the additive combination of the invention in reducing steel corrosion and in improving the oxidation resistance of ester base lubricants, Compositions VII, VIII, IX, and X were subjected to a 75 Bearing Rig test under Type 1½ conditions as set forth

in U.S. Military Specification MIL-L-23699. Specification limits and test results are recorded in the following table.

TABLE II

| Bearing Rig Test, 100 hrs.<br>Type I and 1½ | MIL-L-23699<br>Limits | Composition |       |      |       |
|---------------------------------------------|-----------------------|-------------|-------|------|-------|
|                                             |                       | VII         | VIII  | IX   | X     |
| Bearing dermetit rating                     | 10.7                  | 12.0        | 3     | 6.8  |       |
| Overall dermetit rating                     | 80 max                | 36.6        | 38.6  | 16   | 19.2  |
| Filter deposits, g.                         | 3.0 max               | 0.63        | 0.72  | 0.80 | 0.78  |
| Viscosity change, 100° F.,<br>percent       | -5 to +25             | 228.7       | 114.4 | 24.3 | 22.7  |
| Acid number change                          | 2.0 max               | 7.54        | 6.98  | 0.52 | 0.58  |
| Oil consumption, ml.                        | 2,000 max             | 2,089       | 2,103 | 970  | 1,540 |
| Soluble iron content, p.p.m.                |                       | 366         | 174   | 2.9  | 6.3   |

The foregoing data clearly illustrate the surprising advantages of the inventive compositions (Compositions IX and X) over those containing an acid-amine salt alone (Composition VII), or a combination of an acid-amine salt with a triaryl phosphate (Composition VIII). While Composition VIII does have somewhat improved properties in respect to viscosity index change and soluble iron content, it can be seen that Compositions IX and X containing the additive combination of the invention are markedly superior to the other compositions tested. This difference exceeds that which would be expected by taking a sum of the individual additives performances, indicating that there is a beneficial coaction between the three additives which contributes to the unexpected properties.

### EXAMPLE III

In Table III are presented results of further soluble iron content determinations on Compositions I and II after a series of nine Type 1½ Bearing Rig test runs. Also shown are the load-carrying capacities of these compositions as determined by means of the Ryder Gear test. A complete description of this latter test may be found in ASTM Bulletin No. 184, p. 41, September 1952.

TABLE III

| Test procedure                                                                                             | Composition |       |
|------------------------------------------------------------------------------------------------------------|-------------|-------|
|                                                                                                            | I           | II    |
| Soluble iron content after type 1½ bearing testing (average of results obtained on nine test runs), p.p.m. | 137         | 12    |
| Ryder Gear Test, load-carrying capacity, lbs./in.                                                          | 3,640       | 3,955 |

The relatively low concentration of dissolved iron in Composition II prepared in accordance with the invention, as compared to Composition I containing only an acid-amine salt, is a further indication of effectiveness of the present compositions in preventing steel corrosion. The Ryder Gear Test results demonstrate that there is also a complementary reaction between the additives of the invention in respect to load-carrying capacity. This is evident since Additive B and Additive C by themselves do not possess any significant extreme-pressure activity as indicated by the data in Table IV infra, yet when combined with the acid-amine salt (Additive A) there is a substantial increase in load-carrying exceeding that of Composition I containing a larger amount of Additive A alone.

### EXAMPLE IV

To demonstrate further the efficacy of the present additive combination in improving the load-carrying properties of ester base fluids, Compositions III, IV, V, and VI were also subjected to the Ryder Gear test. Compositions III, IV, and V contained equal concentrations of Additive A, B, and C respectively, while composition VI prepared in accordance with the invention contained an equal total concentration, i.e., 1.22% w. of the combined additives. The base oils used in the preparation of these blends were identical.

In addition, the aforementioned compositions were evaluated by means of the new Thermal Stability-Corrosivity Test which is set forth as part of the proposed MIL-L-23699-B U.S. Navy Specification. Results of these tests are presented in the following tabulation.

TABLE IV

| Test procedure                                              | Composition |       |       |       |
|-------------------------------------------------------------|-------------|-------|-------|-------|
|                                                             | III         | IV    | V     | VI    |
| Ryder Gear Test, load-carrying capacity, lbs./in.:          |             |       |       |       |
| A side                                                      | 2,260       | 4,030 | 2,330 | 3,750 |
| B side                                                      | 2,500       | 3,680 | 2,420 | 3,250 |
| Average                                                     | 2,380       | 3,865 | 2,357 | 3,500 |
| Relative rating, percent                                    | 85.4        | 138.4 | 85.2  | 125.6 |
| Naval Thermal Stability-Corrosivity Test, 525° F., 90 hrs.: |             |       |       |       |
| Iron weight loss, mg.                                       | 1.2         |       |       | 11.5  |
| Viscosity increase, percent                                 | 2.2         |       |       | Nil   |
| TAN-E increase                                              | 2.65        |       |       | 2.49  |

<sup>1</sup> Sample exploded.

25

The data of Table IV further illustrate the increased load-carrying activity derived from the beneficial coaction of the present additives. Although Additives B and C do not impart any significant extreme pressure properties to Compositions III and IV, they markedly improve the loadability of Composition VI, producing a load-carrying-capacity nearly equivalent to that of Composition IV which contains six times more of extreme pressure Additive A than does Composition VI. Compositions IV and V exploded during the Naval Thermal Stability-Corrosivity test indicating acid-amine salts or azelaic acid individually do not impart the requisite stability-corrosivity properties to ester base compositions. When these additives are used in combination with a trihydrocarbyl phosphate, however, a significantly improved product results, possessing excellent extreme-pressure, thermal stability and anticorrosivity properties.

We claim as our invention:

1. A lubricant composition consisting essentially of a major amount of a synthetic carboxylic acid ester lubricating oil and (1) from 0.005 to 10% by weight of a tri-C<sub>1-15</sub> hydrocarbyl phosphate, (2) from 0.005 to 10% by weight of a salt of a C<sub>8-30</sub> primary or secondary alkyl amine and a monohaloalkylphosphonic acid, wherein the haloalkyl radical contains from 1 to 4 carbon atoms, and (3) from 0.001 to 2% by weight of an aliphatic dicarboxylic acid having from 4 to 14 carbon atoms.
2. The composition of claim 1 wherein the phosphate compound is selected from the group consisting of triarylphosphates and trialkaryl phosphates, said aryl and alkaryl groups having from 1 to 10 carbon atoms each.
3. The composition of claim 2 wherein the acid-amine salt is the salt of a monochloroalkylphosphonic acid and an amine selected from the group consisting of primary amines and secondary amines having from 12 to 24 carbons per molecule.
4. The composition of claim 1 wherein the phosphate compound is present in the amount of from 0.01 to 3% by weight, the acid-amine salt is present in the amount of from 0.01 to 2% by weight and the dicarboxylic acid is present in the amount of from 0.01 to 1% by weight.
5. The composition of claim 4 wherein the ester lubricating oil is an ester of monocarboxylic acid having 4 to 14 carbon atoms and a polyalcohol selected from the group consisting of pentaerythritol, dipentaerythritol, trimethylolpropane and mixtures thereof.
6. The composition of claim 5 wherein the phosphate compound is tricresyl phosphate.
7. The composition of claim 6 wherein the acid-amine

salt is the salt of monochloromethyl phosphonic acid and a C<sub>18-22</sub> tertiary alkyl primary amine.

8. The composition of claim 7 wherein the dicarboxylic acid is azelaic acid.

9. The composition of claim 8 wherein the ester base oil is a mixture of C<sub>4-10</sub> monocarboxylic acid esters of pentaerythritol and dipentaerythritol.

3,160,657 12/1964 Price et al. ----- 252-32.5 X  
3,505,230 4/1970 Thompson ----- 252-565

## OTHER REFERENCES

DANIEL E. WYMAN, Primary Examiner

W. H. CANNON, Assistant Examiner

## References Cited

## UNITED STATES PATENTS

2,858,332 10/1958 Watson et al. ----- 252-32.5 X  
2,938,871 5/1960 Matuszak et al. ----- 252-49.9

10

5 Egan, "Lubrication Engineering" March-February 1947,  
pp. 24, 25 and 26.

U.S. Cl. X.R.